

## UNITED STATES PATENT OFFICE

2,254,490

## LUBRICANT

John M. Musselman, South Euclid, Ohio, assignor  
to The Standard Oil Company, Cleveland, Ohio,  
a corporation of Ohio

No Drawing. Application July 7, 1939,  
Serial No. 283,251

6 Claims. (Cl. 252—34)

Lubricating oil in high temperature usage such as in internal combustion engines is subjected to drastic conditions which break down the oil and very greatly limit the durability of an oil which under more ordinary conditions of usage would maintain satisfactory properties. Efforts at improvement by incorporation of certain nitrogen compounds have been made. I have however found that a combination of certain diaryl compounds with certain halogenated carboxylic acids, in such lubricating oils shows remarkable durability over lubricants heretofore known. This is all the more surprising, in view of the fact that the action of such carboxylic acid per se with the oil is without useful effect, while the effect of my new combination is out of all proportion to the sum of the constituents.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

The oil may be of such stock and lubricant viscosity as desired, and for instance conveniently a lubricating stock of Mid-Continent type with viscosity 40 to 200 sec. Saybolt Universal at 210° F. The compounds of the diaryl diamines, preferably diaryl ethylenediamines, may be prepared by heating together, (as over a steam bath), the diamine and a halo-carboxylic acid having at least six carbon atoms. Molar proportions of the diamine and of the acid are preferred, although no difficulty results if one component be in excess, there being in such event merely a dilution from the maximum possible. The diaryl ethylenediamine may be for instance symmetrical diphenylethylenediamine, di-o-tolyl ethylenediamine, etc. The halogenated carboxylic acid of at least six carbon atoms may be for instance chlorostearic acid, chloronaphthenic acid, chloropalmitic acid, and the like. Generally, the chlor-compound is preferred. Illustrative are symmetrical diphenylethylenediamine dichlorostearate, symmetrical diphenylethylenediamine chloronaphthenate, symmetrical diphenylethylenediamine dichloropalmitate, di-o-tolyl ethylenediamine dichlorostearate, di-o-tolyl

ethylenediamine dichloropalmitate, di-o-tolyl ethylenediamine chloronaphthenate, etc. Such compound is readily soluble in the oil, and may be incorporated therein in amounts of for instance 0.01 to 5 per cent, but most generally an amount of 0.5 per cent is desirable. In internal combustion engine usage the body of the oil is well maintained, and such difficulties as sticking of piston rings etc. are particularly inhibited.

10 As an example: A Mid-Continent S. A. E. 30 oil is compounded with 0.5 per cent of symmetrical diphenylethylenediamine chloronaphthenate.

15 As another example: With a similar oil there is incorporated 0.5 per cent of di-o-tolyl ethylenediamine dichlorostearate.

As another example: With a similar oil there is incorporated 0.5 per cent of di-o-tolyl ethylenediamine naphthenate.

20 20 As another example: With a similar oil there is incorporated 0.5 per cent of symmetrical diphenylethylenediamine dichlorostearate.

25 Other modes of applying the principle of the invention may be employed, change being made as regards the details described, provided the features stated in any of the following claims, or the equivalent of such, be employed.

I therefore particularly point out and distinctly claim as my invention:

30 1. A lubricating oil containing a small amount of a diaryl ethylenediamine compound of a halogenated carboxylic acid having at least six carbon atoms.

35 2. A lubricating oil containing a small amount of a symmetrical diphenylethylenediamine compound of a halogenated carboxylic acid having at least six carbon atoms.

3. A lubricating oil containing a small amount of a di-o-tolyl ethylenediamine compound of a halogenated carboxylic acid having at least six carbon atoms.

4. A lubricating oil containing a small amount of symmetrical diphenylethylenediamine dichlorostearate.

45 5. A lubricating oil containing a small amount of symmetrical diphenylethylenediamine chloronaphthenate.

6. A lubricating oil containing a small amount of di-o-tolyl ethylenediamine naphthenate.

50

JOHN M. MUSSELMAN.